

## UNITED STATES PATENT OFFICE

2,293,640

## PROCESS OF CONCENTRATING PHOSPHATE MINERALS

Arthur Crago, Mulberry, Fla., assignor to Phosphate Recovery Corporation, New York, N. Y., a corporation of Delaware

No Drawing. Application October 8, 1940,  
Serial No. 360,261

11 Claims. (Cl. 209—166)

The present invention relates to concentration of phosphate minerals from their ores.

The methods of concentration which are being extensively practiced for the concentration of phosphate minerals in Florida and elsewhere depend on the use of an agent of the negative-ion or anionic active type for preferential collection of the phosphate values in the ore. While phosphate concentrates of commercial grades are obtained by such methods of concentration, they are sometimes obtained with difficulty and only with the sacrifice of recovery; that is, in the practicing of these methods on a commercial scale, when conditions are so adjusted as to yield high grade concentrates, a considerable percentage of the phosphate values in the ore is often not collected and therefore goes to waste with the tailings.

The general object of the invention is to provide an improved method of concentration which will be economical and practical and which will not only facilitate the production of concentrates of high grade, but will also result in the recovery of a high percentage of the phosphate values in the ore.

The invention is the result of the discovery that excellent results as to both grade and recovery may be obtained, with economy, by first subjecting the phosphate ore to a concentrating operation with a negative-ion agent to collect and remove therefrom a rougher concentrate containing a high proportion of the phosphate values mixed with some silicious gangue, and thereafter subjecting this rougher concentrate, after removal of the negative-ion agent, to a concentrating operation with a positive-ion agent to collect and remove therefrom most of the contained silicious gangue. The first concentrating step of the method can be carried out in such a manner as to collect almost the whole of the phosphate present in the ore but the rough concentrate so obtained will contain a good deal of silica. In recleaning such a rough concentrate by conventional means much of the phosphate accompanies the rejected silica and therefore does not appear in the finished concentrate. By submitting the rough concentrates to the second concentrating step of my new process, however, the silicious impurities removed are accompanied by very little phosphate. Since the rougher concentrates contain very little silica as compared with the original ore, only very small quantities of positive-ion agent are required. In such small quantities, as I have discovered, the positive-ion agent gives remarkable results from the

standpoint of selectivity without loss in collecting power; that is, it collects almost no phosphate and a very high percentage of the silicious impurities from the rougher concentrate.

5 By this invention, it is economically possible not only to obtain recoveries, in the form of finished concentrates, considerably exceeding the recoveries obtained by prior methods of concentration, but the finished concentrates are of improved grade because of more thorough separation of the impurities in the ore.

In the carrying out of either of the two concentrating operations made use of by the invention, any concentrating device may be used which 15 is capable of discharging the collected material in such forms as floating froth, skin or surface float, individual agglomerates, etc. Among such devices are included flotation machines and gravity-concentrating tables, the collected material being discharged in the case of the former in the form of a floating froth over the lip of the machine, and in the case of the latter in the form of skin float and suspended agglomerates at the table side.

20 Examples of negative-ion agents which may be used in the carrying out of the first concentrating operation are the higher fatty acids, such as fish oil fatty acid and oleic acid and their soaps, the resin acids and their soaps, wood by-

25 product fatty acids, naphthenic acids and their salts, the higher sulpho-fatty acids and their salts with the proper bases, the acid esters of high-molecular-weight aliphatic alcohols with inorganic acids and their alkali-metal and alka-

30 line-earth-metal salts, the higher xanthates, etc. Examples of positive-ion agents which may be used in the carrying out of the second concentrating operation are the higher aliphatic amines and their salts with water-soluble acids,

35 the esters of amino-alcohols with high-molecular-weight fatty acids and their salts with water-soluble acids, the higher alkyl-O-substituted isoureas and their salts with water-soluble acids, the resin amines and their salts with water-solu-

40 ble acids, the higher aliphatic quaternary ammonium bases and their salts with water-soluble acids, the higher alkyl pyridinium salts of water-soluble acids, the higher alkyl quinolinium salts of water-soluble acids, etc. These various exam-

45 ples of negative-ion and positive-ion agents are not, of course, equally effective or useful in the process of the present invention. The use of an anionic active fatty acid compound is preferred in the carrying out of the first concentrating operation, while the use of a cationic active amine

compound is preferred in the carrying out of the second concentrating operation.

It is to be understood that the expressions "concentrating operation with a negative-ion agent" and "concentrating operation with a positive-ion agent" are used herein in their broadest sense to include all agents which it may be deemed desirable to employ in the carrying out of these two concentrating operations. The concentrating operation with a negative-ion agent should generally be carried out by employing the negative-ion agent with its usual cooperating substances, namely, mineral oil and alkali. The concentrating operation with a positive-ion agent may be carried out in the absence of additional substances, although the use of mineral oil along with the positive-ion agent frequently may be found of advantage for the purpose of agglomeration. It may also be desirable in some instances to use the positive-ion agent in a state of solution in an organic solvent. In froth flotation, of course, either of the two concentrating operations may be carried out with the additional use of a suitable frother.

As an intermediate step between the two concentrating operations, the process of the present invention includes a removal of the effect which the negative-ion agent treatment employed in the first concentrating operation would otherwise have on the second concentrating operation carried out by positive-ion agent treatment. This intermediate step particularly aims to remove the effect of the negative-ion agent treatment from the phosphate values recovered in the rougher concentrate, which values otherwise have the tendency to be separated with the remaining impurities in the second concentrating operation; it being understood that this intermediate step not only removes the effect of the negative-ion agent itself, but also removes the effect of all other associated agents used in the first concentrating operation. It may, of course, be carried out in various ways, it being sufficient in most instances to treat the rougher concentrate for a suitable period with a mineral acid, preferably sulphuric acid.

Some positive-ion agents are known to operate best when added to thin pulps and quickly distributed therein. This is true, for example, of the higher aliphatic amines, as well as of their salts with water-soluble acids. When use is made, in the process of the present invention, of positive-ion agents of this character, no preconditioning or preliminary agitation of the rougher concentrate in their presence is required; that is, they may be added directly to the dilute pulp undergoing separation of the remaining impurities.

In preparing the ore for treatment by the process of the present invention, it is in general desirable that it be comminuted to a particle size most suitable for efficient operation, and that it be largely deslimed thereby minimizing the consumption of the reagents. Ordinarily, the crude ore is first subjected to a preliminary grinding operation and thereafter screened or classified to remove all particles other than those desired. The undersize may then be deslimed, and the oversize reground, deslimed, and added to the deslimed undersize; or the oversize may be reground, added to the undeslimed undersize, and the whole then deslimed.

For a clearer understanding of the invention, certain tests will now be described. These con-

sisted of two series, namely, a first series of three tests and a second series of two tests. Only the second series of tests should be regarded as being pertinent to the invention, the first series being carried out entirely in accordance with known procedures of concentration by negative-ion agent treatment to afford a basis of comparison with the second. Each series was carried out on a sample of minus 35-mesh flotation feed from plant No. 2 of the Phosphate Recovery Corporation in Florida, consisting mainly of so-called bone phosphate of lime (tri-calcium phosphate) and silica sand, the B. P. L. (bone phosphate of lime) content of the sample being about 31%.

15

#### Tests 1 to 3

Each of these three tests was carried out as follows:

The ore in the form of a thick aqueous pulp of about 70% solids was agitated in an impeller-type mixer with fish oil fatty acid, fuel oil, and caustic soda. These three reagents were added during agitation to the mixer, their addition requiring about one minute, after which agitation in the mixer was continued for two more minutes. The pulp conditioned in this manner was transferred to a subaeration flotation machine where, in a diluted state, it was frothed for one minute, during which a rougher concentrate of the phosphate values was floated off. With the tailing removed, this rougher concentrate was returned to the flotation machine where, without further addition of reagents, it was again treated for a period of one minute to float off a finished concentrate.

The results of the three tests are indicated in the following table, which gives the reagent quantities employed in each instance in pounds per ton (2000 lbs.) of dry material treated.

| Test No. | Reagents in lbs. per ton |          |              | Finished concentrate   |                    |                           |
|----------|--------------------------|----------|--------------|------------------------|--------------------|---------------------------|
|          | Fatty acid               | Fuel oil | Caustic soda | Percent B. P. L. assay | Percent Ins. assay | Percent B. P. L. recovery |
| 1.....   | 1.02                     | 2.62     | 0.70         | 75.04                  | 5.12               | 77.7                      |
| 2.....   | 0.71                     | 2.03     | 0.60         | 75.54                  | 3.57               | 58.6                      |
| 3.....   | 0.51                     | 1.84     | 0.50         | 76.14                  | 3.02               | 47.3                      |

As will be noted, the reagents in test 1 were employed in the highest amounts, which resulted in a 77.7% B. P. L. recovery in a finished concentrate assaying 75.04% B. P. L. The lesser reagent amounts of test 2 caused an increase of concentrate grade to 75.54% B. P. L., but a drop in B. P. L. recovery to 58.6%. The still lesser reagent amounts of test 3 caused a further increase of concentrate grade to 76.14% B. P. L., but a further drop in B. P. L. recovery to 47.3%. It is clear that the finished concentrate obtained in test 1 was the best obtainable without unduly lowering the recovery. No advantage would have been gained by increasing the reagent amounts used in test 1, which would simply have raised the recovery with a lowering in grade.

#### Tests 4 and 5

Each of these two tests was carried out as follows:

In the same manner as before, a rougher concentrate was first produced with fish oil fatty acid, fuel oil, and caustic soda. This rougher concentrate was agitated for two minutes with sulphuric acid to remove the effect of these agents, the contaminated liquor obtained by this acid

treatment being removed by decantation. The rougher concentrate was then returned to the flotation machine where it was formed with water into a dilute pulp of about 25% solids and, without preliminary agitation, frothed for one minute in the presence of octadecylamine acetate. Almost pure silica was floated off in this operation, the material remaining in the machine constituting the finished concentrate.

The results of these two tests are shown in the following table, the reagent amounts being again given in pounds per ton (2000 lbs.) of dry material treated.

5 ing the ore in aqueous pulp to a concentrating operation in the presence of an anionic active fatty acid compound, a mineral oil and an alkali to separate a collected material consisting of a rougher concentrate of the phosphate values admixed with entrained silicious gangue, treating the rougher concentrate with a mineral acid to remove the effect of the agents used in its production, and subjecting this rougher concentrate in aqueous pulp to a concentrating operation in the presence of a cationic active amine compound which is a selective collector for the gangue in said rougher concentrate to separate

| Test No. | Reagents in lbs. per ton |          |              |                                               | Finished concentrate           |                        |                    |      |
|----------|--------------------------|----------|--------------|-----------------------------------------------|--------------------------------|------------------------|--------------------|------|
|          | Rougher float            |          |              | Acid treatment H <sub>2</sub> SO <sub>4</sub> | Final float amine <sup>1</sup> | Percent B. P. L. assay | Percent Ins. assay |      |
|          | Fatty acid               | Fuel oil | Caustic soda |                                               |                                | Percent B. P. L. rec.  |                    |      |
| 4        | 1.04                     | 2.62     | 0.70         | 2.00                                          | 0.20                           | 77.14                  | 1.70               | 79.2 |
| 5        | 1.41                     | 3.69     | 0.70         | 2.00                                          | 0.20                           | 77.14                  | 1.80               | 87.5 |

<sup>1</sup> Octadecylamine acetate.

This table shows that both tests 4 and 5 resulted in finished concentrates of improved grade and improved recovery. These concentrates were of the same grade, namely, 77.14% B. P. L., but differed greatly in recovery, 79.2% B. P. L. being recovered in the finished concentrate of test 4 and 87.5% B. P. L. being recovered in the finished concentrate of test 5. In this connection it will be noted that, while the reagent quantities used in test 4 for the rougher operation, were substantially the same as in test 1, the fatty acid and fuel oil quantities used in test 5 were appreciably greater than in test 1. Therefore, test 5 started out with a much higher recovery in the rougher concentrate than test 4. Although the rougher concentrate of test 5 was of much lower grade than the rougher concentrate of test 4, yet the finished concentrates of the two tests were of the same improved grade by reason of the very efficient removal of silica by octadecylamine acetate. This reagent in each of tests 4 and 5 was used in very small amount, and in this small amount had practically no collecting power for the phosphate values in the rougher concentrate. The recovery effected in each instance in the first concentrating operation was consequently maintained in the second concentrating operation.

It is to be understood that the invention as defined in the appended claims is not limited by any details of the foregoing exposition.

What is claimed is:

1. A method of concentrating phosphate minerals from their ores, which comprises subjecting the ore in aqueous pulp to a concentrating operation with a negative-ion agent to separate a rougher concentrate of the phosphate values admixed with entrained silicious gangue, treating the rougher concentrate with a mineral acid to remove the effect of the negative-ion agent treatment used in its production, and thereafter subjecting the rougher concentrate in aqueous pulp to a concentrating operation with a positive-ion agent which is a selective collector for the gangue in said rougher concentrate to separate a collected material largely composed of the entrained silicious gangue, thereby producing a final phosphate concentrate.

2. A method of concentrating phosphate minerals from their ores, which comprises subject-

35 a collected material largely composed of the entrained silicious gangue, thereby producing a final phosphate concentrate.

3. A method of concentrating phosphate minerals from their ores, which comprises subjecting the ore in aqueous pulp to a concentrating operation in the presence of fish oil fatty acid, fuel oil and caustic soda to separate a collected material consisting of a rougher concentrate of the phosphate values admixed with entrained silicious gangue, treating the rougher concentrate with a mineral acid to remove the effect of the agents used in its production, and subjecting the rougher concentrate in aqueous pulp to a concentrating operation in the presence of octadecylamine acetate to separate a collected material largely composed of the remaining gangue, thereby producing a final phosphate concentrate.

4. A method of concentrating phosphate minerals from their ores, which comprises subjecting the ore in aqueous pulp to a concentrating operation in the presence of oleic acid, fuel oil and caustic soda to separate a collected material consisting of a rougher concentrate of the phosphate values admixed with entrained silicious gangue, treating the rougher concentrate with a mineral acid to remove the effect of the agents used in its production, and subjecting the rougher concentrate in aqueous pulp to a concentrating operation in the presence of octadecylamine acetate to separate a collected material largely composed of the remaining gangue, thereby producing a final phosphate concentrate.

5. A method of concentrating phosphate minerals from their ores, which comprises subjecting the ore in aqueous pulp to a concentrating operation in the presence of fish oil fatty acid, fuel oil and caustic soda to separate a collected material consisting of a rougher concentrate of the phosphate values admixed with entrained silicious gangue, treating the rougher concentrate with sulphuric acid to remove the effect of the agents used in its production, and subjecting the rougher concentrate in aqueous pulp to a concentrating operation in the presence of octadecylamine acetate to separate a collected material largely composed of the remaining gangue, thereby producing a final phosphate concentrate.

6. A method of concentrating phosphate min-

erals from their ores, which comprises subjecting the ore in aqueous pulp to a concentrating operation in the presence of wood by-product fatty acid, fuel oil and caustic soda to separate a collected material consisting of a rougher concentrate of the phosphate values admixed with entrained silicious gangue, treating the rougher concentrate with sulphuric acid to remove the effect of the agents used in its production, and subjecting the rougher concentrate in aqueous pulp to a concentrating operation in the presence of octadecylamine acetate to separate a collected material largely composed of the remaining gangue, thereby producing a final phosphate concentrate.

7. A method of concentrating phosphate minerals from their ores, which comprises subjecting the ore in aqueous pulp to a flotation operation with a negative-ion agent to float off a material consisting of a rougher concentrate of the phosphate values admixed with entrained silicious gangue, treating the rougher concentrate with a mineral acid to remove the effect of the negative-ion agent treatment used in its production, and thereafter subjecting this rougher concentrate in aqueous pulp to a flotation operation with a positive-ion agent which is a selective collector for the gangue in said rougher concentrate to float off a material largely composed of the entrained silicious gangue, thereby producing a final phosphate concentrate.

8. A method of concentrating phosphate minerals from their ores, which comprises subjecting the ore in aqueous pulp to a tabling operation with a negative-ion agent to effect a table side separation of a material consisting of a rougher concentrate of the phosphate values admixed with entrained silicious gangue, treating the rougher concentrate with a mineral acid to remove the effect of the negative-ion agent treatment used in its production, and thereafter subjecting this rougher concentrate to a tabling operation with a positive-ion agent which is a selective collector for the gangue in said rougher concentrate to effect a table side separation of

10 a material largely composed of the entrained silicious gangue, thereby producing a final phosphate concentrate.

9. A method of concentrating phosphate minerals from their ores, which comprises subjecting the ore in aqueous pulp to a concentrating operation with reagents to separate a rougher concentrate of the phosphate values admixed with entrained silicious gangue, treating the rougher concentrate with a mineral acid to remove the effect of the reagents used in its production, and thereafter subjecting the rougher concentrate in aqueous pulp to a concentrating operation to separate a collected material largely composed of the entrained silicious gangue, thereby producing a final phosphate concentrate.

15 10. A method of concentrating phosphate minerals from their ores, which comprises subjecting the ore in aqueous pulp to a flotation operation with reagents to float off a material consisting of a rougher concentrate of the phosphate values admixed with entrained silicious gangue, treating the rougher concentrate with a mineral acid to remove the effect of the reagents used in its production, and thereafter subjecting this rougher concentrate in aqueous pulp to a flotation operation to float off a material largely composed of the entrained silicious gangue, thereby producing a final phosphate concentrate.

20 11. A method of concentrating phosphate minerals from their ores, which comprises subjecting the ore in aqueous pulp to a tabling operation with reagents to effect a table side separation of a material consisting of a rougher concentrate of the phosphate values admixed with entrained silicious gangue, treating the rougher concentrate with a mineral acid to remove the effect of the reagents used in its production, and thereafter subjecting this rougher concentrate to a tabling operation to effect a table side separation of a material largely composed of the entrained silicious gangue, thereby producing a final phosphate concentrate.

30 35 40 45 ARTHUR CRAGO.